

## UNITED STATES PATENT OFFICE

1,928,204

DETONATOR AND COMPOSITION FOR  
THE SAMESylvester B. Large, Tamaqua, Pa., assignor to  
Atlas Powder Company, Wilmington, Del., a  
corporation of DelawareNo Drawing. Application December 15, 1930  
Serial No. 502,559

15 Claims. (Cl. 52—4)

This invention relates to improvements in blasting caps which are used for initiating charges of explosives.

Its object is to provide blasting caps of the compound or booster type which are marked by great economy and by decreased hazard in manufacture and use, but with no sacrifice of efficiency. A further object is the adaptation of an improved type of primary detonating substance as the 10 initiator for the base charge in compound blasting caps. The invention is applicable to either electric or safety fuse types of blasting caps.

Compound blasting caps comprise a base charge of some explosive which is not usually a primary detonating substance in itself. Examples of base charges are tetryl, trinitrotoluene, nitrocellulose; in fact, solid explosives generally are possibilities. The primary detonating or initiating substance for the base charge has, in 20 practice, usually been mercury fulminate or an azide. Confining capsules may be positioned in various parts of the loading, as between the initiator and base charge or above the initiator.

The previously used primary detonating substances have been characterized by extreme sensitivity to impact, friction and handling generally. They are also hazardous in manufacture and quite costly.

I have now found a type of primary detonating substance for compound blasting caps which approaches the ideal. Solid organic nitrates of the general formula  $C_nH_{n+2}(NO_3)_n$ , of which hexanitromannite is an example, have received consideration as admixtures in dynamites, blasting cap compounds, primers and certain military compositions. A well known type of blasting cap may consist of a mixture of mercury fulminate, nitrocellulose, potassium chlorate and hexanitromannite. It has been proposed that a blasting 40 cap be made by pressing a compound of the proposed type in a shell and igniting it with a hot flame composition such as a mixture of barium nitrate, magnesium powder and lead hypophosphate.

45 World-wide tendency has been toward compound blasting caps because of their greater economy, decreased hazard and great efficiency. As a base charge an explosive may be used which is stronger, cheaper, safer and more effective 50 than most primary detonating substances. Most any solid explosive such as tetryl, TNT, nitrocellulose, nitrostarch, hexanitromannite, tetra-nitroerythrite, trinitrobenzene, etc., may be used in this relation. It will be observed that these 55 cited base charges are less sensitive to friction

and impact than mercury fulminate, lead azide and diazodinitrophenol. Tendencies in the use of primary detonating substances for such blasting caps have been toward those of which the lesser amounts are necessary, because of the resultant economy and the decreased amounts of hazardous materials that it is necessary to handle. Thus azides and diazodinitrophenol are replacing mercury fulminate for the above reasons. However, such compounds are all highly hazardous in handling with respect to impact, friction and pressure. The use of decreased quantities involves only a partial elimination of hazard, at the best, while in some of the manufacturing operations it is of no value and results 60 in no hazard elimination whatever, for the user.

65 I have searched repeatedly, and over an extended period, for a primary detonating substance which would be suitable for initiating the base charge in compound blasting caps and would be less hazardous than known compounds for the purpose. In the discovery of the adaptability 70 of compounds of the proposed type, namely organic nitrates of the general formula  $C_nH_{n+2}(NO_3)_n$ , I have been successful beyond 75 expectation. In addition to achieving the stated aims, I have also obtained a higher degree of initiating efficiency than is offered by mercury fulminate and a higher strength than is offered by other known primary detonating substances.

80 In my examples I will refer to tetryl as the base charge and hexanitromannite as the primary detonating substance. This is in no respect limiting since I may use base charges that 85 are suitable with other primary detonating substances and I may use primary detonating substances of the general formula  $C_nH_{n+2}(NO_3)_n$ .

90 In the following table the base charge was always 0.30 gram tetryl pressed at 100# and an 95 inner capsule was used over the hexanitromannite.

| Weight of hexanitromannite | Pressure on hexanitromannite | Lead plates |
|----------------------------|------------------------------|-------------|
| Gram                       | Pounds                       |             |
| .15                        | 50                           | A           |
| .15                        | 100                          | A           |
| .15                        | 150                          | A           |
| .15                        | 200                          | A           |

100

105

The above indicates that under an inner capsule as little as 0.15 gram hexanitromannite will detonate a tetryl base charge, whether the pressure is 50 lbs. or 200 lbs.

110

Some Bureau of Mines type sand tests results were:

| 5  | Weight of tetryl base charge | Tetryl pressed at | Weight of hexanitromannite | Hexanitromannite pressed at | Grams of sand crushed |
|----|------------------------------|-------------------|----------------------------|-----------------------------|-----------------------|
|    | Gram                         | Pounds            | Gram                       | Pounds                      |                       |
| 10 | 0.10                         | No                | 0.25                       | 150                         | 39                    |
|    | 0.15                         | No                | 0.25                       | 150                         | 40½                   |
|    | 0.50                         | 100               | 0.25                       | 150                         | 59                    |
|    | 0.60                         | 100               | 0.25                       | 150                         | 62                    |

It is here indicated that a base charge of 0.15 gram tetryl and a primer charge of 0.25 gram of hexanitromannite is suitable for a No. 6 blasting cap and that a base charge of 0.60 gram tetryl and a primer charge of 0.25 gram hexanitromannite is suitable for a No. 8 blasting cap.

In testing primary detonating substances for frictional sensitiveness one of my tests upon which I place much reliance consisted in placing a small amount of sand in a copper cup, loading the substance on it and pressing with a revolving steel press point, with facilities to record the pressure when detonation occurred. The results in a series of tests were:

| 30 | Primary detonating substances               | Average pressure at which detonation occurred |
|----|---------------------------------------------|-----------------------------------------------|
|    |                                             | Pounds                                        |
| 35 | Mercury fulminate                           | 264                                           |
|    | 80-20 mercury fulminate-potassium chlorate  | 320                                           |
|    | Diazodinitrophenol                          | 340                                           |
|    | 75-25 diazodinitrophenol-potassium chlorate | 240                                           |
|    | Lead azide                                  | 181                                           |
|    | Mercurious azide                            | 215                                           |
|    | Hexanitromannite                            | No explosions at 500                          |

Another test upon which I place much reliance consisted in placing a small amount of the substance on a hardened steel anvil, inclined at a 20° angle and dropping a steel ball weighing approximately 80 grams on the substance; noting the height of fall necessary to cause complete detonation.

Results in a series of tests were:

| 50 | Primary detonating substance                | Minimum height at which detonation occurred |
|----|---------------------------------------------|---------------------------------------------|
|    |                                             | Inches                                      |
| 55 | Mercury fulminate                           | 6                                           |
|    | 80-20 mercury fulminate-potassium chlorate  | 8                                           |
|    | Diazodinitrophenol                          | 6                                           |
|    | 75-25 diazodinitrophenol-potassium chlorate | 10                                          |
|    | Lead azide                                  | 12                                          |
|    | Mercurious azide                            | None at 32                                  |
|    | Hexanitromannite                            |                                             |

60 In this test of hexanitromannite which was made at the maximum height possible with the apparatus, it was noted that some very slight local crackings occurred at the point of contact between the steel ball and the steel anvil. In no case did these slight crackings propagate to the balance of the substance, which is a very desirable feature and of great importance in manufacturing blasting caps.

65 It is indicated in these tests that hexanitromannite presents the least hazard by a wide margin.

An important feature of my present invention resides in the provision of suitable and adequate igniting means for the primary charge. The present application is intended to cover broadly 75 the use of substances having the general for-

mula  $C_nH_{n+2}(NO_3)_n$  as the primary charge in compound detonators, irrespective of the particular igniting means which may be employed. However, it is highly important to employ a suitable and effective ignition means, because, since the material of the primary charge is less sensitive than mercury fulminate and other commonly employed initiators, such insensitivity must be compensated for by the use of particularly reliable and effective igniting means or flash composition. While I do not desire to limit this application to the use of any particular igniting medium, yet, in order to recite a completely operative combination, I may refer to the disclosure of my co-pending application Serial No. 502,560, filed December 15, 1930, the match heads there described having been found by me to be satisfactory igniting mediums for detonators of the character contemplated in this application.

80

The synthetic manufacture of mannite has been developed to a point where it is much cheaper than the same product from natural sources. Accordingly, in consideration of this, together with the fact that such small quantities of nitromannite are requisite for the primary charges thereof, my novel type of compound detonator is believed more economical than any heretofore known or used.

90

It is to be understood that the solid explosive substances of the general formula  $C_nH_{n+2}(NO_3)_n$ , specified as essential to my invention, may be the ordinary grades of impure products usually produced, for example by the nitration of the commercial forms of the required polyhydric alcohols of the general formula  $C_nH_{n+2}(OH)_n$ ; the said nitration products being prone to contain certain impure isomers, lower nitric esters, etc. They may, however, also be the chemically pure compounds, as obtained, for example, by recrystallization of impure forms, from a suitable solvent or solvents. Hexanitromannite, or nitromannite, for example, may refer either to the chemically pure hexanitric ester or it may include proportions of the lower nitric esters, mixed therewith.

100

Having described my invention, which I claim is:

110

1. A compound detonator in which the primary detonating substance is a solid explosive of the general formula  $C_nH_{n+2}(NO_3)_n$ .

115

2. A compound detonator in which the primary detonating substance is a mixture of solid organic nitrates of the general formula  $C_nH_{n+2}(NO_3)_n$ .

120

3. A compound detonator in which the base charge is an explosive which is not a primary detonating substance and upon which is placed a primary charge of a solid composition of the general formula  $C_nH_{n+2}(NO_3)_n$ .

125

4. A compound detonator in which the base charge is a solid explosive which is less sensitive to friction and impact than mercury fulminate, lead azide and diazodinitrophenol and upon which is placed a primary charge of a solid nitration product of the general formula  $C_nH_{n+2}(NO_3)_n$ .

130

5. A compound detonator whose primary charge consists of a solid nitration product of the general formula  $C_nH_{n+2}(NO_3)_n$  and a stabilizing agent.

135

6. A compound detonator consisting of a base charge of tetryl and a primary detonating charge of hexanitromannite.

140

7. A compound detonator comprising a base charge of tetryl and a primary charge consisting of hexanitromannite.

145

8. A compound detonator comprising a base

150

charge and a primary charge having as an essential ingredient hexanitromannite.

9. As a new article of manufacture, a detonator including, in combination, a shell, a base charge 5 of a solid explosive which is less sensitive to friction and impact than mercury fulminate, lead azide and diazodinitrophenol, a primary charge consisting of a mixture of a solid explosive substance of the general formula  $C_nH_{n+2}(NO_3)_n$  and 10 a stabilizing agent, a perforated inner capsule pressed over the said primary charge, and an ignition medium for the said charge.

10. A detonator comprising, in combination, a shell, a base charge of an explosive which is not 15 a primary detonating substance, a primary detonating charge of a solid organic nitrate of the general formula  $C_nH_{n+2}(NO_3)_n$ , a perforated inner capsule pressed over the said primary charge, and a suitable ignition medium for the 20 said charge.

11. A detonator comprising, in combination, a shell, a base charge of an explosive which is less sensitive than mercury fulminate, lead azide and diazodinitrophenol, a primary detonating charge 25 of a mixture of a solid organic nitrate of the

general formula  $C_nH_{n+2}(NO_3)_n$  and a stabilizing agent, a perforated inner capsule pressed over the said primary charge, and a suitable igniting medium for the said charge.

12. A compound detonator including a base 80 charge of tetryl and upon which is placed a primary charge consisting of hexanitromannite and a stabilizing agent.

13. A detonator as recited in claim 9 characterized by having hexanitromannite as the solid explosive constituent of the said primary charge. 85

14. A detonator as recited in claim 9 characterized by having tetryl as the said base charge thereof.

15. A detonator comprising a shell, a base charge of a solid explosive less sensitive to friction and impact than mercury fulminate, lead azide and diazodinitrophenol, a superimposed primary charge of a solid nitration product of the general formula  $C_nH_{n+2}(NO_3)_n$ , and a hot 90 flash material of such composition as to quickly ignite and bring about detonation of the primary charge of  $C_nH_{n+2}(NO_3)_n$ . 95

SYLVESTER B. LARGE. 100

30

105

35

110

40

115

45

120

50

125

55

130

60

135

65

140

70

145

150